

## UNITED STATES PATENT OFFICE.

ALADAR PACZ, OF CLEVELAND, OHIO, ASSIGNOR TO GENERAL ELECTRIC COMPANY, A CORPORATION OF NEW YORK.

## TUNGSTEN ALLOY.

No Drawing. Application filed January 15, 1920; Serial No. 351,684. Renewed January 24, 1923.

To all whom it may concern:

Be it known that I, ALADAR PACZ, a citizen of the United States, residing at Cleveland, in the county of Cuyahoga and State 5 of Ohio, have invented a new and useful Tungsten Alloy, of which the following is a specification.

My invention relates to the production of combinations of tungsten with silicon for 10 use especially for filaments in electric incandescent lamps. I have found that when tungsten is combined with silicon, the latter being present in a comparatively small proportion, exceptionally good results are 15 secured especially when the metal is used for filaments for incandescent lamps.

According to my invention, I prefer to produce the alloy or mixture of tungsten and silicon by first intimately mixing the tungsten with silicic acid and then reducing the latter. One method which may be followed 20 is to mix about 5 grams of powdered magnesium with about 300 grams of finely divided tungsten mixed with about 6 grams of 25 finely divided silicic acid. In my application Serial Number 149,915, filed Feb. 20, 1917, I have described a method of preparing tungsten which includes the preliminary preparation of finely divided tungsten 30 intimately mixed with silicic acid and which is used in the production of the so-called 218 metal. That mixture of tungsten and silicic acid may be utilized to advantage in the present instance. The mixture thus produced may be passed through 35 a highly heated furnace, for instance, an electrically heated furnace, the magnesium reducing the silicic acid to form metallic silicon intimately incorporated with the tungsten powder. The magnesium oxide 40 which forms in the re-action may then be dissolved out by hydrochloric acid leaving only the mixture of the tungsten and the silicon. If preferred, the reduction may be 45 made of tungstic acid mixed with silicic acid, the tungstic acid being reduced by hydrogen and the silicic acid by magnesium. The mixture of tungsten and silicon is 50 pressed into slugs, formed and otherwise mechanically treated and drawn into wire as described in the Coolidge Patent No. 1,082,933.

It is my theory that by the above described method, an alloy or composite metal

of tungsten and silicon is produced in 55 which the silicon is dissolved in the tungsten and the silicon is not volatilized out to the extent that silica is volatilized in the regular 218 process described in the afore- 60 said application.

Incandescent lamp filaments produced from the combination of tungsten and silicon possesses in a high degree, non-sagging qualities like those of the 218 wire and, 65 moreover, do not interlock when the lamp is subjected to shock such as in a bump test. This makes this wire especially suitable for straight filaments although it is also useful for coiled filaments.

The percentages of silicon may vary 70 somewhat but a comparatively small quantity is all that is necessary and I have found that between 1 and 3 per cent silicon in the metal before forming, gives the best results.

What I claim and desire to secure by Letters Patent of the United States is:—

1. A drawn metal filament for electric incandescent lamps consisting of tungsten with which is intimately incorporated a small percentage of silicon.

2. A drawn wire consisting of tungsten with which is intimately incorporated a small percentage of silicon.

3. The process of producing wire suitable for electric incandescent lamp filaments and similar devices, which consists in heating to a high temperature a mixture of a tungsten material, a silicon compound and a reducing agent, pressing the resultant finely divided metal into slugs and subsequently heating and mechanically working the same.

4. A process of producing wire suitable for electric incandescent lamp filaments and similar devices which consists in heating to a high temperature a mixture of a tungsten material, silicic acid and magnesium, pressing the resultant metal into slugs and then heating and mechanically working the same.

5. The process of producing wire suitable for electric incandescent lamp filaments and similar devices which consists in pressing into slugs finely divided tungsten having silicon intimately incorporated therewith and then sintering and mechanically working the same.

In witness whereof I have hereunto set my hand this 26th day of December, 1919.

ALADAR PACZ.